

Aug. 23, 1932.

P. R. BETTISON

1,872,653

FLOOR COVERING

Filed Jan. 18, 1928

Fig. 1.



Fig. 2.



INVENTOR.  
Percy R. Bettison  
BY  
Charles French  
ATTORNEYS

## UNITED STATES PATENT OFFICE

PERCY R. BETTISON, OF CHICAGO, ILLINOIS, ASSIGNOR TO AMERICAN HAIR & FELT COMPANY, OF CHICAGO, ILLINOIS, A CORPORATION OF DELAWARE

## FLOOR COVERING

Application filed January 18, 1928. Serial No. 247,626.

55

The invention relates to floor coverings and more particularly to those floor coverings commonly known as linoleums and to a method of producing the same.

5 The usual linoleum floor covering consists of a mastic formed of ground cork or wood-meal, whose particles are secured together by a suitable cement, such as linoxyn or its substitutes, and is spread upon a fabric base. 10 This floor covering as such is relatively hard and unyielding and is generally laid on hard surfaced flooring. It is also difficult, laborious and expensive to lay the linoleum upon a yieldable floor covering. The object of 15 this invention is to provide a floor covering in which a yieldable or cushion base is formed during the process of making the linoleum floor covering and more particularly a floor covering comprising linoleum mastic incorporated with a fabric base which 20 forms a part of a cushion layer of punched felt so that the linoleum surface and the felt form a unitary flooring material.

The invention further consists in the several features hereinafter set forth and more particularly defined by claims at the conclusion hereof.

In the drawing Fig. 1 is a vertical sectional view through a floor covering embodying the invention;

30 Fig. 2 is a similar view showing a modification.

Referring to the drawing, in each instance the numeral 3 designates the linoleum mastic, 35 4 a fabric layer, such as burlap, 5 a layer of fibrous cushioning material, preferably felt, the fibres of which are loosely felted together and then punch felted to the burlap 4 so that a sheet of punched felt is formed.

40 The punched felt with the strip of burlap attached is then run over one of two calender rolls by means of which the prepared mastic is caused to flow over the burlap to the punched felt upon the fabric-backed side 45 thereof and is then cured in the usual

manner so that the mastic is intimately associated with the fabric and parts of the fibres of felt that project through the interstices of the fabric. The felt may be formed from any suitable vegetable or 60 animal fibre but preferably consists principally of animal hair which is more resilient than vegetable fibres and maintains its resiliency. The resulting product is a linoleum having a cushioned bottom which provides a 65 yieldable tread surface. This product may be readily secured to the harder surfaced flooring by cementing the felt thereto, but to further improve upon the bond between the flooring and the cement, I have shown, in 70 Fig. 2, an additional fabric bottom layer 6 which is secured to the fibrous material by punching the fibres through it.

My floor covering is adaptable for completely covering floors, as they are ordinarily 75 covered with linoleum, or for partially covering the floor, as is customary with rugs; it may be made into rugs, strips, or any desirable form. In some cases the floor covering may be cemented to the floor and in other 80 cases it may be desirable not to have it cemented. This method of use is optional.

In the drawing the felt layer 5 is shown as thicker than the linoleum mastic layer 3. This need not be the case. In fact, in practice I prefer to have the felt layer of less 85 thickness than the linoleum.

I desire it to be understood that this invention is not to be limited to any particular form or arrangement of parts except insofar 90 as such limitations are included in the claims.

What I claim as my invention is:

1. As a new article of manufacture, a floor covering comprising a fabric layer, a layer of feltable fibres secured thereto, and a 95 layer of linoleum mastic sheeted onto said fabric layer and cured thereon.

2. As a new article of manufacture, a floor covering comprising a fabric layer, a layer of feltable fibres punch-felted thereto, 100

and a layer of linoleum mastic sheeted on said fabric layer and cured thereon.

3. As a new article of manufacture, a floor covering comprising a fabric layer, a layer of feltable fibres punch-felted thereto, **5** a layer of linoleum mastic sheeted onto said fabric layer and cured thereon, and a bottom fabric layer secured to the bottom face of said layer of feltable fibres.

10 In testimony whereof, I affix my signature.  
**PERCY R. BETTISON.**

**15****20****25****30****35****40****45****50****55****60**